# EUROPEAN PATENT SPECIFICATION

(11) **EP 0 232 015 B1**
(45) Date of publication and mention of the grant of the patent: **12.12.1990**
(21) Application number: 87300212.5
(22) Date of filing: 09.01.1987
(51) Int. Cl.: D21H 17/46

(54) **Pitch control aid**
Hilfsmittel zur Harzkontrolle
Agent auxiliaire pour le contrôle de la poix

(30) Priority: 09.01.1986 GB 8600506
(43) Date of publication of application: 12.08.1987
(73) Proprietor: W.R. Grace AB, S-25 106 Helsingborg (SE)
(72) Inventor: Hassler, Thord Gustav Gunnar, S-253 72 Helsingborg (SE)
(74) Representative: Ellis-Jones, Patrick George Armine

(56) References cited:
- CA-A- 1 150 914
- US-A- 3 855 299
- US-E- 28 808

## Description

This invention relates to the control of pitch in the manufacture of pulp and paper.

It is well known that "pitch" can accumulate in paper making and also in the manufacture of pulp, causing significant problems. "Pitch" is the term used to describe the sticky materials which appear in paper making; these originate from the wood from which the paper is made. However, nowadays when more recycled paper is used, "pitch" is now used as a general term for all material soluble in organic solvents but not soluble in water, for example the ink or adhesive present in recycled paper. The pitch can accumulate at various points in the system. For example, it can block the felt and thus hinder drainage of the paper web. In addition, it can adhere to the wires or drying cylinders causing it to pick holes in the paper. Deposits may also build up at any earlier stage in the papermaking process. When these deposits break loose they may form a defect in the paper such as a spot or a hole. Such defects may even create a weakness in the paper sufficient to induce a breakage in the paper during the production resulting in unappreciated production down-time.

Many materials have been used in an attempt to eliminate these problems. Such materials include inorganic treatments such as talc and anionic dispersants. However, conventional dispersants can be ineffective in a closed system as there can be a build-up of "pitch". In such systems the pitch particles have to be removed from the water system in a controlled way without being allowed to accumulate on the felt or rolls or, for example, the pipe work used in the paper making machinery. These products have also been found to give a limited effect and there is a need for further improved treatments.

It has now been found, according to the present invention, that certain water soluble poly-quaternary amines are particularly effective for this purpose. Accordingly, the present invention provides a method for the control of pitch in an aqueous system used during pulp or paper making which comprises adding to the system or to the pulp making or paper making machinery, a water soluble poly-quaternary branched polymer derived from (a) an epihalohydrin, a diepoxide or a precursor of an epihalohydrin or diepoxide, (b) an alkyl amine having a functionality with respect to an epihalohydrin of two, and (c) ammonia or an amine which has a functionality with respect to an epihalohydrin greater than two and which does not possess any carbonyl groups, with one or more of the following conditions:

(i) the polymer is added to the pulp making or paper making machinery, (ii) the pulp is of recycled paper containing adhesive, and (iii) components (a) and (b) are reacted to form a coupling agent which is then reacted with component (c).

A special feature of the products used in the present invention is that they may combine with dissolved anionic material originating from the wood from which the pulp and paper is produced, providing a method of removing these anionic materials thereby lowering the concentration of such materials in the process water. Water soluble anionic materials are released from the wood during pulp manufacture. These components interfere with paper production negatively in several ways: they decrease the efficiency of many products used in the papermaking process to alter the character of the paper. Examples of such additives include sizes, wet and dry strength agents and dyes. Anionic dissolved materials also reduce the efficiency of retention agents. They limit the extent to which the water system can be closed and they may also lower the quality of the paper such as its strength. Reference is made to TAPPI papermakers Conference 1979 p49-66 which further discusses, the significance of anionic dissolved materials.

Component (a) is preferably an epihalohydrin, especially epichlorohydrin or epibromohydrin, but dihalohydrins, preferably dichlorohydrins or dibromohydrins, having three to twenty, especially three to ten, carbon atoms per molecule may also be used. Typical dihalohydrins which may be used include the following:
CH₂CICHCICH₂0H
CH₂CICH₂(OH)CH₂CI
CH₃CHCICHCICH₂0H
CH₃CHCICH(OH)CH₂CI
CH₃CH₂CHCICHCICH₂0H
CH₃CHCICHCICH(OH)CH₃
CH₃CH₂CHCICH(OH)CI
CH₃CH₂CH(OH)CHCICH₂CI
CH₃CHCICH(OH)CHCICH₃ and

As regards component (b) the alkyl amine may be a compound possessing two tertiary amino groups such as N,N,N',N'-tetramethyleneethylenediamine. Details of the preparation of products derived from such component (b) and component (a) can be found in UK-A-1 486 396. However, component (b) is preferably a dialkylamine in which the alkyl groups individually contain one to three atoms. Dimethylamine is especially preferred.

As previously indicated, component (c) is ammonia or an amine which possesses a functionality greater than two with respect to epihalohydrin and which does not possess any carbonyl groups; it can therefore act as a branching agent. It has been found that the use of a branched polymer is an important feature in the performance of the polymer to prevent deposition of pitch, as the comparative experiments below show. A primary amino group is capable of reacting with three molecules of epihalohydrin so that a simple primary amine possesses a functionality of three. Likewise, a simple secondary amine will possess a functionality of two and a simple tertiary amine a functionality of one. Accordingly, component (c) is typically ammonia, a primary amine, a primary alkylene polyamine having four to twenty-five, preferably four to twelve, carbon atoms and at least one, preferably one to six, primary amino groups per molecule including polyglycolamines as well as aromatic and heteroaromatic diamines but not polyamidoamines because they possess carbonyl groups. Preferred materials include ammonia, diethylaminobutylamine, dimethylaminopropylamine and ethylenediamine, the latter two being especially preferred.

If desired, the polymer may also be derived from a further component which generally has the ability to act as a "end-capping" agent. In general, these materials will also be amines or other material having reactivity towards epichlorohydrin and which possess a functionality less than two and which also possess some other functional group or a fatty chain of, say, at least 12 carbon atoms, such as a simple tertiary amine such as a trialkylamine, especially trimethylamine or a hydroxyalkylamine, typically triethanolamine, or a fatty amine such as octadecylamine.

The polymers used in the present invention may be prepared by first reacting components (a) and (b) to obtain a "coupling agent" and then reacting this with component (c) and, if desired, the fourth component. Preferred polymers for use in the present invention include those in which the coupling agent is derived from epichlorohydrin and dimethylamine, which is subsequently reacted with ethylenediamine and, if desired, also with trimethylamine, triethanolamine or octadecylamine.

The polymers may also be prepared by reacting a mixture of components (b) and (c) with component (a). The preferred raw materials for such a process are the same as those given above.

In general, the reaction is carried out in an aqueous medium, typically maintaining the reaction temperature at 5 to 125_{°}C, preferably 30 to 95_{°}C The equivalent ratio of component (b) to component (c) is suitably 1:0.009 to 1.0 and preferably 1:0.02 to 0.5 while the equivalent ratio of component (a) to components (b) and (c) may vary widely depending on the amount and nature of component (b). Generally, the ratio of component (c) to component (a) and component (b), together should be selected so that the viscosity of the aqueous polymer solution is at least 20 mPa - (Cps) at 50% dry content. Typically, the ratio is from 1:0.22 to 2.5 and preferably 1:0.25 to 1.3. In general, the reaction can be continued until the desired viscosity, and therefore molecular weight, has been achieved although acid can be used to reduce the pH and thereby terminate the reaction. A pH of I to 7.5, especially 2 to 6.5, is generally preferred for the final solution.

The upper viscosity limit is not critical provided it is consistent with having a workable solution; the upper limit is normally about 2000 mPa . (Cps).

Further details regarding the polymers which can be used and their preparation is to be found in, inter alia, UK-A-2 085 433, US-A-3 855 299 and US Patent Re-Issue 28 808 and, for certain polymers, in "Polyelectrolytes for Water and Wastewater Treatment", ed W L K Schwoyer, CRC Press Inc, pages 26 - 35. A particularly preferred polymer for use in the present invention is formed by reacting ethylenediamine with a precondensate of dimethylamine and epichlorohydrin, and reacting the product with triethanolamine to form a water-soluble reaction product. Another preferred product is formed by reacting a mixture of dimethylamine and ethylenediamine or dimethylaminopropylamine with epichlorohydrin to form a water-soluble reaction product.

The polymer is generally added to the aqueous system with the furnish containing the paper pulp but it is possible to add it at different points in the system depending on the precise nature of the problem.

The amount of polymer required will, of course, depend to some extent on the nature of the wood or other material used to prepare the paper pulp. Also, some polymer once added will tend to recirculate in the system thus requiring a lower addition rate. In general, however, from 0.1 to 20 ppm of polymer by weight based on the aqueous medium is suitable. Preferably, the amount is I to 10 ppm. This corresponds in the normal case to an addition of 10 to 2,000 grams, preferably 100 to 1,000 grams, polymer per tonne fibre. However, in cases where the polymer is required to neutralize anionic dissolved materials, generally higher amounts are desirable, in the normal case from 1,000 grams to 50,000, especially from 1,500 to 15,000 grams, per tonne fibre depending on the process by which the fibres are produced (see, for example, Progr. Colloid & Polymer Sci. 65, 251-264 (1978) for a discusssion of the amounts of anionic material likely to be present). Fibres produced by a mechanical process generally require a higher addition than fibre prepared by a chemical process. It is, of course, also possible to only partly neutralize the total amount of dissolved anionic materials. In such cases amounts from as little as, say, 10 grams per tonne of paper may be effective.

Sometimes it can be preferred to spray the reaction product used in this invention onto a particular part of the pulp- or paper-making machinery such as the wire or press felts. In such cases, the polymer is preferably pre-diluted with water, generally to a concentration below 10% by weight and preferably I to 5% by weight.

In some instances, it will be convenient to add the polymer together with a biocide. Examples of suitable biocides include those in the following classes:
(i) a substituted 5- or 6-membered ring heterocyclic compound in which the hetero atom or atoms are one or more of nitrogen, oxygen or sulphur and the substituent is an alkyl group, a keto group or a hydroxyl group or a halogen atom, such compounds include isothiazolones, and in particular, those having the formula: wherein R represents hydrogen or chlorine. A blend of these two isothiazolones is commercially available, the weight ratio of the chloro-substituted compound to the unsubstituted compound being about 2.66:1;
(ii) a phenol or chlorinated phenol such as pentachlorophenol;
(iii) an amine or amide including 2,2-dibromo-3-nitrilopropionamide;
(iv) an organic cyanide or thiocyanate, particularly methylene bis(thiocyanates);
(v) a sulphone including halosulphones, particularly hexachlorodimethylsulphone;
(vi) a straight chain aliphatic aldehyde, particularly glutaraldehyde;
(vii) a triazine, particularly thio and/or amino-substituted alkyl triazines;
(viii) bis bromo acetoxy butene; and
(ix) a dithiocarbamate, especially the monomethyl, dimethyl, monoethyl and diethyl derivatives, typically in the form of sodium salts.

The polymer is generally compatible with the usual pulp and paper making additives including starch, for example potato or corn starch, titanium dioxide, a defoamer such as a fatty acid alcohol, a size, for example a rosin size based on abietic acid, a neutral size based on alkyl ketene dimer or a succinic acid anhydride based size and a wet strength resin such as, if neutral, an epichlorohydrin polyamide or, if acid, a melamine- or urea-formaldehyde resin.

The precise nature of the pH of the system is unimportant since the effectiveness of the polymer is substantially unaffected by changes in pH.

Some of the polymers used in the present invention are commercially available, typically as aqueous solutions containing a concentration of 40 to 50% per cent. Typically, the compositions used in the present invention will possess from I to 70%, especially 10 to 30%, by weight of the polymer.

The following examples further illustrate the present invention.

### EXAMPLE

Into a reaction flask fitted with reflux condenser, mechanical stirrer and thermometer were placed 183.5 g of 32.7% dimethylamine and 270g of water. 76.04 g of 36% hydrochloric acid was added while maintaining a temperature maximum of 35_{°}C by cooling. 208.12 g epichlorohydrin was added during 30 minutes. Cooling was applied to keep the temperature not above 40_{°}C. This temperature was maintained for two hours to produce a stock solution of so-called "coupling agent". 176.9 g of the aqueous solution of the coupling agent was, using the same equipment, heated to 60°C. 5.94 g of ethylenediamine was added dropwise over a 30 minute period. The temperature was then kept at 60_{°}C for one hour. The reaction mixture was heated to 90_{°}C and 32.48 g of 30% trimethylamine was added during ten minutes; 90_{°}C was then maintained for two hours and the reaction mixture cooled to room temperature. This reaction mixture had a total solids content of 40.7%.

### EXAMPLE 2

Using the equipment described in Example I, 25.35 g of 36% hydrochloric acid was added to a mixture of 68.81 g of 32.7% dimethylamine solution and 121.4 g water. The temperature was kept below 35°C by cooling. 83.25 g epichlorohydrin was added at such a rate that temperature was maintained at 40_{°}C. This temperature was then kept for one hour. The reaction mixture was heated to 60_{°}C and 7.5 g ethylene diamine was added over 15 minutes while maintaining the temperature at 60_{°}C. This temperature was kept for another 30 minutes. The reaction mixture was heated to 90_{°}C and 37.25 g triethanolamine was added dropwise over 30 minutes. This temperature was maintained for a further two hours to complete the reaction. The total solids content was 44.6%.

### EXAMPLE 3

The products prepared in Examples I and 2 were evaluated using essentially the method described in 1977 TAPPI paper makers Conference p 23-32 by Ch E Farley. This method is built on TAPPI Standard Method RC324 which is a recognised method for evaluating depositability of pitch. The standard pitch solution was prepared as described in the above references. A synthetic pitch emulsion/dispersion was prepared by adding one litre volume of deionised water at 50_{°}C to the synthetic pitch to reach a 1200 ppm concentration.

A solution of calcium chloride was added to reach a hardness of 340 ppm expressed as calcium carbonate. The pH was adjusted to 8.0. To evaluate the products as pitch control agents, the products were added to obtain a concentration of polymer as specified in Table I. The depositability of the pitch was evaluated according to the procedure in the above references. The test duration was always five minutes. The results are presented in Table I (mg deposited pitch).

### COMPARATIVE EXAMPLE I

An aminoplast resin was prepared essentially according to Example III in US Patent 3 582 461 for comparison.

84 g (I mole) of dicyandiamide, 196 (2.4 moles) of 37% by weight inhibited aqueous formaldehyde solution, 126 g (mole) of 85% active formic acid were charged into a I litre four neck flask equipped with an agitator, thermometer and condenser. The mixture was agitated for 0.5 hours at room temperature. External heat was applied to the reaction mixture and the mixture was heated to 60°C over a 0.5 hour period. The reaction temperature was gradually raised from 60_{°}C to the boiling point of the mixture. The exothermic reaction, which occurred when the temperature was raised above 60_{°}C, was controlled by intermittent cooling. The boiling point of the reaction mixture was reached after three hours heating. The mixture was boiled for 15 minutes and then cooled rapidly to 55_{°}C. 42 g of methanol was added to etherify free methylol groups and the mixture was agitated for 2.5 hours and then cooled to 25_{°}C. The resulting reaction product was a water soluble dicyandiamide-formaldehyde condensate in the form of a clear water soluble syrup containing 40% by weight solids.

This resin was evaluated according to procedure in Example 3 with the following results.

### COMPARATIVE EXAMPLE 2

Some other products with potential as pitch control agents were evaluated following the procedure of Example 3 with the following results.

### EXAMPLE 4

. To a mixture of 68.81 g of 32.7% dimethylamine and 121.4 g water was added 25.35 g of 36% hydrochloric acid dropwise over 30 minutes. The temperature of the reaction mixture was not allowed to exceed 35_{°}C; some cooling was required. 83.25 g of epichlorohydrin was added at such a rate that the temperature of the reaction mixture was maintained at 40_{°}C. After the exothermic reaction was completed the solution was maintained at 40_{°}C until it became clear (I hour). After heating to 60_{°}C, 7.5 g of ethylenediamine was added quickly over 5 minutes. The reaction mixture was maintained at 65_{°}C for a further hour. The reaction mixture was then cooled to room temperature. To 97.42 g of this solution was added 22.56 g octadecylamine (2 moles) and 7.5 g 2-methoxy ethanol (to assist solution). This slurry was slowly heated to 70_{°}C and maintained at this temperature for 30 minutes. Further heating to 75_{°}C produced a highly exothermic reaction which required external cooling to maintain a temperature of 75_{°}C. After completion of the exothermic reaction, the mixture was heated at 90°C for 2 hours. The product, which was in the form of a creamy emulsion, had a total solid content of 18%.

### EXAMPLE 5

The product of Example 4 was evaluated using the method described in Example 3, but a different synthetic pitch was used. This time a pitch solution was made by adding a mixture of 2.0 g tall oil and 20.0 g glycerol ester of rosin to 10.5 g 5% potassium hydroxide to form an emulsion. This was then diluted with 187.5 g isopropanol and 110 g acetone to form a clear pitch solution. 15 ml of this solution was added to one litre water at 20_{°}C and a hardness of 200 ppm expressed as calcium carbonate. The pH was adjusted to 3.0 using concentrated hydrochloric acid and the test was carried out over three minutes.

### COMPARATIVE EXAMPLE 3

Polydiallyl dimethyl ammonium chloride (poly DADMAC) is another poly quaternary resin suggested as a pitch control agent, in European Patent Application 58 621. This resin was tested following the procedure in Example 5.

### COMPARATIVE EXAMPLE 4

The preferred type of quaternary compound for control of pitch deposition in US-A-3 619 351 is a meth- yltriethanolamine. This material was synthesized from triethanolamine and dimethyl sulphate to form quaternary ammonium methyl triethanolamine monomethyl sulphate. This material was evaluated using the procedure in Example 3 with the following results:

### COMPARATIVE EXAMPLE 5

A resin was prepared only from dimethylamine and epichlorohydrin following essentially the procedure of Example I of US reissue 28,807. A 500 ml round bottom flask equipped with condenser, mechanical stirrer, thermometer and pH electrodes was used for the preparation. 92.5 grams (1.0 mole) epichlorohydrin was added to the flask. 112.5 grams of 40% aqueous dimethylamine (45 grams real, 1.0 mole) was added with vigorous stirring over one hour keeping the temperature below 50_{°}C. Heating was applied for another two hours at 50_{°}C whereafter 70g water was added. The viscosity of this resin was determined to be 72 mPa- s (cps) and dry content was found to be 47 percent.

### EXAMPLE 6

The same equipment as in Comparative Example 5 was used; 63.5 g water, 9g ethylenediamine and 121.9g aqueous solution (36.9%) of dimethylamine was added to the reaction flask. 170g epichlorohydrin was added over a three hour period maintaining the temperature below 35_{°}C by cooling. Temperature was then increased to 80_{°}C. 11.8g epichlorohydrin was added in six portions over three hours and after the last addition the reaction mass was kept at 80_{°}C for an additional two hours, whereafter the product was cooled to room temperature. The product was a pale yellow slightly opaque liquid with a dry content of 65.8% and a viscosity of 190 mPa· s (cps).

### EXAMPLE 7

The same equipment as in Comparative Example 5 was used. Water (34.2g), dimethylamine (60.9g of an aqueous 36.9% solution) and ethylenediamine (1.5g) were charged to the reaction flask. 5I.0g epichlorohydrin was added with vigorous stirring over 2 hours. Temperature was raised to 80_{°}C and 10.6g epichlorohydrin was added in 9 portions over a 8 hour period. The final product was a slightly opaque, pale yellow liquid. Dry content of this product was found to be 58.8% and the viscosity approx 1000 mPa (cps).

### EXAMPLE 8

The equipment of Comparative Example 5 was used. A resin was prepared in the following way: 112.5 grams 40% dimethylamine was added to the reaction flask together with 10.2 grams dimethylaminopropylamine. These two amines were mixed and 102 grams of epichlorohydrin was added over 30 minutes with vigorous stirring maintaining a temperature of 30-40°C. Temperature was then increased to 60_{°}C which was maintained for 5 hours. During this period of time, 300ml of deionised water was added in small portions. This resin had a viscosity of 20 mPa s (cps) and a dry content of 33%.

### EXAMPLE 9

The products of Comparative Example 5 and Examples 6 to 8 were evaluated following the procedure of Example 5 at an addition of I.0ppm polymer with the following results:

### EXAMPLE 10

The resin of Example 6 was evaluated using the method of Example 3. The following results were obtained:

### EXAMPLE 11

In order to evaluate the usefulness of polymers to combine with anionic dissolved components of paper pulp the following experiment was made:
A dried groundwood pulp from pine was disintegrated for 30 minutes to prepare a 2.5% furnish. The fibres were subsequently filtered off and the filtrate was used to evaluate the capacity of the resins to combine with dissolved anionic materials. The amount of anionic material was determined with a streaming current detector. Polyethyleneimine (PEI) was used as standard. The efficiency to combine with anionic material was evaluated by adding to the filtrate various amounts of resin, stirring for 15 minutes and subsequently determining the residual concentration of uncombined anionic material by titration with the standard reagent. The results were as follows:

## Claims

1. A method for the control of pitch in an aqueous system used during pulp or paper making which comprises adding to the system, or to the pulp making or paper making machinery, a water soluble poly-quaternary branched polymer derived from (a) an epihalohydrin, a diepoxide or a precursor of an epihalohydrin or diepoxide, (b) an alkyl amine having a functionality with respect to an epihalohydrin of 2 and (c) ammonia or an amine which has a functionality with respect to an epihalohydrin greater than 2 and which does not possess any carbonyl groups, with one or more of the following conditions:
(i) the polymer is added to the pulp making or paper making machinery,
(ii) the pulp is of recycled paper containing adhesive, and
(iii) components (a) and (b) are reacted to form a coupling agent which is then reacted with component (c).

2. A method according to claim 1 in which component (a) is epichlorohydrin or epibromohydrin.

3. A method according to claim 1 or 2 in which component (b) is a dialkyl amine in which the alkyl groups individually contain 1 to 3 carbon atoms.

4. A method according to claim 3 in which component (b) is dimethylamine.

5. A method according to any one of the preceding claims in which component (c) is a primary amine or a primary alkylene polyamine.

6. A method according to claim 5 in which component (c) is diethylaminobutylamine, dimethylamino-propylamine or ethylene diamine.

7. A method according to any one of the preceding claims in which the polymer is also derived from a tertiary amine or a hydroxy alkyl amine.

8. A method according to claim 7 in which the polymer is also derived from trimethyl amine or triethanol amine.

9. A method according to any one of the preceding claims in which the polymer is one formed by reacting ethylene diamine with a precondensate of dimethyl amine and epichlorohydrin and reacting the product with triethanolamine to form a water soluble reaction product.

10. A method according to any one of claims 1 to 8 in which the polymer is one formed by reacting a mixture of dimethylamine and ethylene diamine or dimethylamino propylamine with epichlorohydrin to form a water soluble reaction product.

11. A method according to any one of the preceding claims in which the equivalent ratio of component (c) to components (a) and (b) together is from 1:0.22 to 2.5.

12. A method according to any one of the preceding claims in which the polymer is added to the aqueous system with the furnish containing the paper pulp.

13. A method according to any one of the preceding claims in which the polymer is added in an amount from 1,000 to 50,000 grams per tonne of fibre.

14. A method according to any one of claims, to 11 in which the polymer is sprayed onto at least a part of the paper making machinery during paper making.

15. A method according to claim 14 in which the polymer is sprayed onto the paper making wires.

16. A method according to claim 14 or 15 in which the polymer is applied as an aqueous solution having a polymer concentration below 10 per cent by weight.

17. A method according to claim 16 in which the polymer concentration is 1 to 5 per cent by weight.

18. A method according to any one of the preceding claims in which the paper making process uses recycled paper containing adhesive.

19. A method according to any one of the preceding claims in which a biocide is also added.

## Patentansprüche

1. Verfahren zur Kontrolle von Harzablagerungen in einem wäßrigen System, das bei der Zellstoff-oder Papierherstellung verwendet wird, bei dem dem System oder der Zellstoffherstellungs- oder Papierherstellungsanlage ein wasserlösliches poly-quaternäres verzweigtes Polymer zugesetzt wird, das sich von (a) einem Epihalohydrin, einem Diepoxid oder einem Vorläufer eines Epihalohydrins oder Diepoxids, (b) einem Alkylamin mit einer Funktionalität bezüglich eines Epihalohydrins von 2 und (c) Ammoniak oder einem Amin, das eine Funkionalität bezüglich eines Epihalohydrins von mehr als 2 aufweist und keine Carbonylgruppen besitzt, bei einer oder mehreren der folgenden Bedingungen ableitet:
(i) das Polymer wird der Zellstoffherstellungs- oder Papierherstellungsanlage zugesetzt,
(ii) der Zellstoff ist aus zurückgeführtem, Klebstoff enthaltendem Papier und
(iii) die Komponenten (a) und (b) werden zur Bildung eines Kupplungsmittels miteinander umgesetzt, welches dann mit Komponente (C) umgesetzt wird.

2. Verfahren nach Anspruch 1, bei dem Komponente (a) Epichlorhydrin oder Epibromhydrin ist.

3. Verfahren nach Anspruch 1 oder 2, bei dem Komponente (b) ein Dialkylamin ist, bei dem die Alkylgruppen individuell 1 bis 3 Kohlenstoffatome enthalten.

4. Verfahren nach Anspruch 3, bei dem Komponente (b) Dimethylamin ist.

5. Verfahren nach einem der vorangehenden Ansprüche, bei dem Komponente (c) ein primäres Amin oder ein primäres Alkylenpolyamin ist.

6. Verfahren nach Anspruch 5, bei dem Komponente (c) Diethylaminobutylamin, DimethylaminoPropylamin oder Ethylendiamin ist.

7. Verfahren nach einem der vorangehenden Ansprüche, bei dem das Polymer sich außerdem von einem tertiären Amin oder einem Hydroxyalkylamin ableitet.

8. Verfahren nach Anspruch 7, bei dem das Polymer sich außerdem von Trimethylamin oder Triethanolamin ableitet.

9. Verfahren nach einem der vorangehenden Ansprüche, bei das Polymer ein solches ist, das durch Umsetzung von Ethylendiamin mit einem Vorkondensat aus Dimethylamin und Epichlorhydrin und Umsetzung des Produkts mit Triethanolamin zur Bildung eines wasserlöslichen Reaktionsprodukts gebildet ist.

10. Verfahren nach einem der Ansprüche 1 bis 8, bei dem das Polymer ein solches ist, das durch Umsetzung einer Mischung von Dimethylamin und Ethylendiamin oder Dimethylaminopropylamin mit Epichlorhydrin zur Bildung eines wasserlöslichen Reaktionsprodukts gebildet ist.

11. Verfahren nach einem der vorangehenden Ansprüche, bei dem das Equivalentverhältnis von Komponente (c) zu Komponenten (a) und (b) zusammen 1:0,22 bis 2,5 beträgt.

12. Verfahren nach einem der vorangehenden Ansprüche, bei dem das Polymer dem wäßrigen System mit der die Papierpulpe enthaltenden Stoffzusammensetzung zugesetzt wird.

13. Verfahren nach einem der vorangehenden Ansprüche, bei dem das Polymer in einer Menge von 1000 bis 50 000 g je Tonne Fasern zugesetzt wird.

14. Verfahren nach einem der Ansprüche 1 bis 11, bei dem das Polymer bei der Papierherstellung zumindest auf einen Teil der Papierherstellungsanlage gesprüht wird.

15. Verfahren nach Anspruch 14, bei dem das Polymer auf das Papierherstellungssieb gesprüht wird.

16. Verfahren nach Anspruch 14 oder 15, bei dem das Polymer als wäßrige Lösung mit einer Polymerkonzentration unterhalb 10 Gew.% angewendet wird.

17. Verfahren nach Anspruch 16, bei dem die Polymerkonzentration 1 bis 5 Gew.% beträgt.

18. Verfahren nach einem der vorangehenden Ansprüche, bei dem das Papierherstellungsverfahren zurückgeführtes, Klebstoff enthaltendes Papier verwendet.

19. Verfahren nach einem der vorangehenden Ansprüche, bei dem außerdem ein Biozid zugesetzt wird.

## Revendications

1. Procédé pour le contrôle de poids dans un système aqueux utilisé pendant la fabrication de la pâte à papier ou du papier, qui comprend l'addition au système, ou à la machinerie de fabrication de papier ou de fabrication de pâte à papier, d'un polymère ramifié polyquaternaire soluble dans l'eau dérivé (a) d'un épihalohydrine, d'un diépoxyde ou d'un précurseur d'un épihalohydrine ou d'un diépoxyde, (b) d'une amine alkyle ayant une fonctionnalité en ce qui concerne un épihalohydrine de deux et (c) de l'ammoniac ou une amine qui a une fonctionnalité en ce qui concerne un épihalohydrine supérieure à deux et qui ne possède aucun groupements carbonyles, acec une ou plusieurs des conditions suivantes :
(i) le polymère est ajouté à la machinerie de fabrication de papier ou de pâte à papier,
(ii) la pâte à papier est un adhésif contenant du papier recyclé, et
(iii) des composants (a) et (b) ont réagi pour former un agent couplant qui ensuite réagi avec le composant (c).

2. Procédé selon la revendication 1, dans lequel le composant (a) est un épichlorohydrine ou un épi- bromohydrine.

3. Procédé selon la revendication 1 ou 2, dans lequel le composant (b) est une amine dialkyle dans laquelle les groupements alkyle contiennent individuellement de 1 à 3 atomes de carbone.

4. Procédé selon la revendication 3, dans lequel le composant (b) est une diméthylamine.

5. Procédé selon l'une quelconque des revendications précédentes, dans lequel le composant (c) est une amine primaire ou une polyamine alkylène primaire.

6. Procédé selon la revendication 5, dans lequel le composant (c) est une diéthylaminobutylamine, une diméthylamino-propylamine ou une éthylène diamine.

7. Procédé selon l'une quelconque des revendications précédentes, dans lequel le polymère est également dérivé d'une amine tertiaire ou d'une hydroxyalkylamine.

8. Procédé selon la revendication 7, dans lequel le polymère est aussi dérivé d'une triméthyle amine ou d'une triéthanolamine.

9. Procédé selon l'une quelconque des revendications précédentes, dans lequel le polymère est celui formé par la réaction d'une éthylène diamine avec un précondensat d'une diméthylamine et d'épichlorohydrine et par la réaction du produit avec la triéthanolamine pour former un produit de réaction soluble dans l'eau.

10. Procédé selon l'une quelconque des revendications 1 à 8, caractérisé en ce que le polymère est celui formé par la réaction d'un mélange de diméthylamine et d'éthylène diamine ou de diméthylaminopropyl- amine avec de l'épichlorohydrine pour former un produit de réaction soluble dans l'eau.

11. Procédé selon l'une quelconque des revendications précédentes, dans lequel le rapport équivalent du composant (c) aux composants (a) et (b) ensemble, est de 1:0,22 à 2,5.

12. Procédé selon l'une quelconque des revendications précédentes, dans lequel le polymère est ajouté au système aqueux avec la matière première contenant la pâte de papier.

13. Procédé selon l'une quelconque des revendications précédentes, dans lequel le polymère est ajouté dans une quantité allant de 1000 à 50 000 grammes par tonne de fibre.

14. Procédé selon l'une quelconque des revendications 1 à 11, dans lequel le polymère est pulvérisé sur au moins une partie de la machinerie fabriquant le papier pendant la fabrication du papier.

15. Procédé selon la revendication 14, dans lequel le polymère est pulvérisé sur les fils métalliques fabriquant le papier.

16. Procédé selon la revendication 14 ou 15, dans lequel le polymère est appliqué comme une solution aqueuse ayant une concentration de polymère au-dessous de 10% en poids.

17. Procédé selon la revendication 16, dans lequel la concentration de polymère est de 1 à 5% en poids.

18. Procédé selon l'une quelconque des revendications précédentes, dans lequel le procédé de fabrication de papier utilise l'adhésif contenant du papier recyclé.

19. Procédé selon l'une quelconque des revendications précédentes, dans lequel un biocide est aussi ajouté.
